# EUROPEAN PATENT SPECIFICATION

(11) **EP 1 645 651 B1**
(45) Date of publication and mention of the grant of the patent: **01.07.2009**
(21) Application number: 04726905.5
(22) Date of filing: 12.04.2004
(51) Int. Cl.: C22F 1/06

(54) **METHOD FOR PRODUCING MAGNESIUM BASE ALLOY FORMED ARTICLE**
VERFAHREN ZUR HERSTELLUNG VON FORMKÖRPERN AUS MAGNESIUMBASISLEGIERUNG
PROCEDE DE PRODUCTION D'ARTICLE EN ALLIAGE DE MAGNESIUM

(30) Priority: 30.05.2003 JP 2003155476
(43) Date of publication of application: 12.04.2006
(73) Proprietor: Sumitomo Electric Industries, Ltd., Osaka-shi, Osaka 541-0041 (JP)
(72) Inventor: OISHI, Yukihiro c/o Itami Works, Itami-shi, Hyogo 6640016 (JP); KAWABE, Nozomu c/o Itami Works, Itami-shi, Hyogo 6640016 (JP)
(74) Representative: Cross, Rupert Edward Blount
(86) International application number: PCT/JP2004/005226
(87) International publication number: WO 2004/106576

(56) References cited:
- JP-A- 60 149 751
- JP-A- 63 282 232
- JP-A- 2001 071 037
- JP-A- 2002 371 334
- JP-A- 2003 293 069
- JP-A- 2004 017 114
- TAKAHASHI H ET AL: "TENSILE PROPERTIES AND BENDING FORMABILITY OF DRAWN MAGNESIUM ALLOY PIPES" MATERIALS SCIENCE FORUM, AEDERMANNSFDORF, CH, vol. 419-422, 2003, pages 345-348, XP009044106 ISSN: 0255-5476
- KOHZU, M. (OSAKA PREFECTURE UNIVERSITY (JAPAN)) ET AL: "Evaluation of press formability in magnesium alloy." MATERIALS SCIENCE FORUM , VOL. 419-422, (PART 1), PP. 321-326, GRAPHS, PHOTOMICROGRAPHS, 7 REF. . SWITZERLAND CONFERENCE: PROCEEDINGS OF THE SECOND OSAKA INTERNATIONAL CONFERENCE ON PLATFORM SCIENCE AND TECHNOLOGY FOR ADVANCED MAGNESIUM ALLOYS 2003,, 2003, XP009081487
- KANEKO J ET AL: "Magnesium gokin tenshinzai no kikai-teki seishitsu to seikei-sei ni oyobosu shugo soshiki no eikyo /EFFECT OF TEXTURE ON THE MECHANICAL PROPERTIES AND FORMABILITY OF MAGNESIUM WROUGHT MATERIALS" NIPPON KINZOKU GAKKAISHI - JOURNAL OF THE JAPAN INSTITUTE OF METALS, NIPPON KINZOKU GAKKAI, TOKYO, JP, vol. 64, no. 2, 2000, pages 141-147, XP002975479 ISSN: 0021-4876
- OISHI Y. ET AL.: 'Kokyodo magnesium gokin wire no kaihatsu' SEI TECHNICAL REVIEW no. 162, February 2003, pages 57 - 61, XP002983073

## Description

### Technical Field

The present invention relates to a method for producing a wrought product made of magnesium-based alloy by plastic processing. More particularly, the invention relates to a producing method of a magnesium-based alloy wrought product capable of producing the wrought product with more excellent productivity while lowering a processing temperature when the plastic working is carried out.

### Background Technique

The magnesium-based alloy is lighter than aluminum in weight, and has more excellent specific strength and specific rigidity as compared with steel or aluminum and thus, the magnesium-based alloy is widely used for aircraft parts, automobile parts, bodies of various electrical products and the like.

However, since Mg and its alloy have hexagonal close-packed lattice (hcp) structure, they have poor ductility and their plastic workability is extremely poor. It is widely known that workability of magnesium-based alloy becomes excellent if the temperature is increased at the time of processing. For example, Japanese Patent Applications Laid-open Nos.2000-283134 and 2000-343178 describe technique for processing a screw in a temperature state in which magnesium-based alloy material generates superplasticity phenomenon.

When magnesium-based alloy material is plastically processed, however, since the temperature at which the superplasticity phenomenon is generated is as high as 250°C or higher, the conventional method has a problem that a wrought product can not be produced by the plastic processing with excellent productivity.

Conventionally, when severe processing such as plastic processing is to be carried out to obtain a wrought product made of magnesium-based alloy, although conditions differ depending upon processing degree, it is necessary to heat extruded material or rolled material made of magnesium-based alloy which is to be processed to 250°C or higher and to process the material. Therefore, heat equipment for high temperature as high as 250°C or higher is not only required, but a mold used for the plastic processing and a processing material such as a roll are also exposed to high temperature and their lifetimes are shortened, and this increases the processing cost. Thus, it is by no means preferable for industrial production to heat material to 250°C or higher. Takahashi, H. et al., 'Tensile Properties and Bending Formability of Drawn Magnesium Alloy Pipes', Mat. Sci. Forum Vols, 419-422 (2003), pp. 345-348, discloses the magnesium alloy pipes may be bent after they have been drawn.

It is a main object ot the present invention to provide a producing method of a magnesium-based alloy wrought product capable of producing a plastically processed wrought product made of magnesium-based alloy with excellent productivity.

### Disclosure of the Invention

It is generally considered it difficult to carry out severe processing such as plastic processing for magnesium-based alloy. The present inventors variously researched and found that if a magnesium-based alloy material which is previously subjected to specific drawing processing is used, plastic processing can be carried out even if the processing temperature is less than 250°C, and achieved the present invention.

That is, the producing method of a magnesium-based alloy wrought product of the present invention is **characterized in that** a drawn material made of magnesium-based alloy obtained by drawing processing is subjected to plastic processing into a wrought product at a processing temperature of less than 250°C.

Conventionally, when a magnesium-based alloy material is subjected to plastic processing to obtain a wrought product, extruded material or rolled material is used as material to be processed. However, if the extruded material or rolled material is used, it must be heated to 250°C or higher at the time of plastic processing, and it is strongly desired to lower the processing temperature. The present invention lowers the processing temperature by using not extruded material or rolled material but a drawn material obtained by the drawing processing, i.e., the invention realizes a plastic processing at less than 250°C, especially at 200°C or lower. According to the invention, it is possible to lower the processing temperature at the time of plastic processing to less than 250°C by using a drawn material, the conventional high temperature heating means is unnecessary, lifetime of a processing material such as a mold or roll used for the plastic processing can be increased, and productivity can be enhanced. The present invention will be explained in more detail.

Examples of the drawn material made of magnesium-based alloy of the invention are a wire (line-like body), a rod-like body, a pipe and the like. A cross section of the drawn material may be of circular, rectangular, non-circular such as elliptic shape, i.e., the cross section may be of any shape.

When a wire or a rod-like body is to be obtained for example, the drawing conditions of the present invention are that a temperature rising speed to the processing temperature is 1°C/sec to 100°C/sec, processing temperature is 50°C or higher and 200°C or lower (more preferably 150°C or lower), processing degree is 10% or more per one drawing processing (one pass), linear speed is 1 m/sec or more, and extruded material or rolled material is drawn. For example, when a pipe is to be obtained, the drawing temperature is 50°C or higher and 300°C or lower (more preferably 100°C or higher and 200°C or lower, and further preferably 100°C or higher and 150°C or lower), processing degree is 5% or higher per one drawing processing (preferably 10% or higher and more preferably 20% or higher), temperature rising speed to the drawing temperature is 1°C/sec to 100°C/sec, drawing speed is 1 m/sec or more, and extruded material or rolled material is drawn. If such a particular drawing processing is carried out, the crystal grain can be fine, and more particularly, the average crystal particle diameter can be reduced to 10µm or less. According to the present invention, by fine grain, the plastic workability can be enhanced even if the heating temperature is less than 250°C, and a desired wrought product can be obtained. After the drawing processing, the obtained drawn material may be heated to temperature of 100°C or higher and 300°C or lower, more preferably 150°C or higher and 300°C or lower. This heating annealing is effective for recovery of lattice defect introduced by the drawing processing, and for further finely dividing crystal grain by acceleration of recrystallization. It is preferable that keeping time of this heating temperature is about 5 to 20 minutes.

The type of plastic processing of the invention are forging processing, swaging processing, bending processing and the like. When the forging processing is to be carried out as the plastic processing, the following temperature conditions are suitable. That is, when reduction in height is r₁% and processing temperature is T°C, T satisfies the relation of 3r₁+150 > T ≥ 3r₁+10 (however, 20% ≤ r₁ < 80%, T < 250°C). For example, when reduction in height r₁ is equal to 20(%), the heating temperature T (°C) is lower than 250°C, especially 70°C or higher and lower than 210°C. When extruded material or rolled material which is not subjected to drawing processing is subjected to forging processing of reduction in height of 20%, crack or the like is generated and forging processing can not be carried out if the material is not heated to high temperature as high as 210°C or higher, but if the material is heated to such high temperature, the lifetime of a processing material such as a mold or roll is shortened. According to the present invention, the heating temperature when forging processing of reduction in height of 20% is carried out can be less than 210°C by the finely dividing effect of alloy structure using drawn material, and the lifetime of a processing material such as a mold or roll can be increased. When processing having reduction in height r₁ of more than 33% is to be carried out, the lower limit value of the heating temperature is set to a value obtained by the 3r₁+10, and the upper limit value of the heating temperature is set to lower than 250°C while taking the lifetime of a mold or roll into consideration. Therefore, according to the present invention, when plastic processing having reduction in height of more than 40% which is industrially effective processing is to be carried out, even if the processing temperature is lower than 250°C, forging processing can sufficiently be carried out. In the severe processing in which reduction in height is 80% or higher, it is desired to heat the material to 250°C or higher.

When swaging processing is to be carried out as the plastic processing, the following temperature conditions are suitable. That is, when cross section reduction ratio is r₂% and processing temperature is T°C, T satisfies the relation of 3r₂+150 > T ≥ 3r₂-30 (however, 20% ≤ r₂ ≤ 80%, T < 250°C). For example, when cross section reduction ratio r₂ is 20%, the heating temperature T (°C) can be less than 250°C, especially 30°C or higher and less than 210°C. Therefore, if the cross section reduction ratio is 20%, according to the present invention in which drawn material having fine alloy structure is used, lifetime of a processing material such as a mold can be increased in comparison with the conventional method in which extruded material or rolled material which is not subjected to drawing processing is used and heating to 210°C or higher is required. When cross section reduction ratio r₂ exceeds 33%, the lower limit value of the heating temperature is set to value obtained by the 3r₂-30, and the upper limit value of the heating temperature is set to lower than 250°C while taking the lifetime of a mold or the like into consideration. In the present invention in which drawn material having fine alloy structure is used, when processing whose cross section reduction ratio exceeds 40% which is industrially effective processing is to be carried out, the swaging processing can be carried out at the processing temperature lower than 250°C. In the severe processing in which cross section reduction ratio exceeds 80%, it is desired to heat the material to 250°C or higher.

When the bending processing is to be carried out as the plastic processing, the following temperature conditions are suitable. That is, if thickness of a drawn material at the time of bending is t mm and bending radius is R mm and processing temperature is T°C, T satisfies (1) 250 > T ≥ 250-250R/t when 0.1 ≤ R/t ≤ 1.0, (2) 500-250R/t ≥ T > 0 when 1.0 < R/t ≤ 1.9, and (3) 25 ≥ T > 0 when 1.9 < R/t ≤ 2.0. For example, when a ratio R/t of bending radius R and thickness t of the drawn material is 1.0 to 1.9, the heating temperature T (°C) can be lower than 250°C, and especially the upper limit value can be 500-250R/t or lower. That is, as will be found from a later-described test result, the heating temperature can be lower than 100°C, further room temperature (e.g., 20°C). When R/t is 1.9 to 2.0, the heating temperature T (°C) can be 25°C or lower. In the conventional method in which extruded material or rolled material which is not subjected to drawing processing is used, if bending processing in which R/t is 1.0 to 2.0, especially about 1.5 to 1.0 is to be carried out, it is necessary to heat the material. On the other hand, according to the present invention, bending processing can sufficiently be carried out with R/t of 1.0 to 2.0 without heating the material due to the effect of fine crystal grain because drawn material is used, and heating equipment is unnecessary. Since heating operation is not necessary, lifetime of a processing material such as a mold can be increased. In the case of severe processing having R/t of less than 1.0, the lower limit value of the heating temperature is set to a value obtained by the 250-250R/t, and the upper limit value of the heating temperature is set to a value lower than 250°C while taking the lifetime of a mold or the like into consideration. According to the conventional method using extruded material, it is necessary to heat the material to 200°C or higher in the severe processing having R/t of 1.2 or less, and especially in the case of severe processing having R/t of 1.0 or less, it is necessary to heat the material to 250°C or higher. Whereas, according to the present invention, since the drawn material in which crystal grain is fine is used, bending processing can sufficiently be carried out at the processing temperature of lower than 250°C even if the bending processing is severe processing in which R/t is 0.1 to 1.0.

The thickness of the drawn material is a diameter when the drawn material is a wire (line-like body) or a rod-like body and its cross sectional shape is circular, a thickness when the drawn material is a wire or a rod-like body and its cross sectional shape is rectangular, and a difference between an outer diameter and an inner diameter when the drawn material is a pipe.

If R/t exceeds 2.0, the degree of the bending processing is low, and even extruded material or rolled material can be processed at room temperature and thus, it is not defined in the present invention. In the case of severe processing in which R/t is less than 0.1, since it is desired to heat the material to higher than 225°C, it is not defined in the present invention while taking the lifetime of a processing material such as a mold into consideration.

The present invention is effective in magnesium-based alloy having hcp structure having poor workability at around roomtemperature (e.g., 20°C) irrespective of alloy composition. For example, casting magnesium-based alloy or flatting magnesium-based alloy can be used. Concrete examples of the alloy are one having 0.1% by weight or more and 12% by weight or less Al and one having 0.1% by weight or more and 10% by weight or less Zn and 0.1% by weight or more and 2.0% by weight or less Zr. When the alloy contains Al, it may contain one or more of 0.1% by weight or more and 2.0% by weight or less Mn, 0.1% by weight or more and 5.0% by weight or less Zn, and 0.1% by weight or more and 5.0% by weight or less Si. As the alloy composition, it is possible to use AZ-based alloy, AS-based alloy, AM-based alloy, ZK-based alloy and the like in representative ASTM symbols. As contents of Al, 0.1 to less than 2.0% by weight Al and more than 2.0 to 12.0% by weight Al may be distinguished from each other. In addition to the above chemical compositions, it is general to use alloy including Mg and impurities. Examples of the impurities are Fe, Si, Cu, Ni, Ca and the like.

Examples of the AZ-based alloy having 2.0 to 12.0% by weight Al are AZ31, AZ61, AZ91 and the like. The AZ31 is a magnesium-based alloy, for example, containing Al: 2.5 to 3.5% by weight, Zn: 0.5 to 1.5% by weight, Mn: 0.15 to 0.5% by weight, Cu: 0.05% by weight or less, Si: 0.1% by weight or less, and Ca: 0.04% by weight or less. The AZ61 is a magnesium-based alloy, for example, containing Al: 5.5 to 7.2% by weight, Zn: 0.4 to 1.5% by weight, Mn: 0.15 to 0.35% by weight, Ni: 0.05% by weight or less, and Si: 0.1% by weight or less. The AZ91 is a magnesium-based alloy, for example, containing Al: 8.1 to 9.7% by weight, Zn: 0.35 to 1.0% by weight, Mn: 0.13% by weight or more, Cu: 0.1% by weight or less, Ni: 0.03% by weight or less, and Si: 0.5% by weight or less. The AZ-based alloy contains Al: 0.1 to less than 2.0% by weight, and examples of the AZ-based alloy are AZ10,AZ21 and the like. The AZ10 is a magnesium-based alloy, for example, containing Al: 1.0 to 1.5% by weight, Zn: 0.2 to 0.6% by weight, Mn: 0.2% by weight or more, Cu: 0.1% by weight or less, Si: 0.1% by weight or less, and Ca: 0.4% by weight or less. The AZ21 is a magnesium-based alloy, for example, containing Al: 1.4 to 2.6% by weight, Zn: 0.5 to 1.5% by weight, Mn: 0.15 to 0.35% by weight, Ni: 0.03% by weight or less, and Si: 0.1% by weight or less.

Examples of the AS-based alloy having Al of 2.0 to 12.0% by weight are AS41 and the like. The AS41 is a magnesium-based alloy, for example, containing Al: 3.7 to 4.8% by weight, Zn: 0.1% by weight or less, Cu: 0.15% by weight or less, Mn: 0.35 to 0.60% by weight, Ni: 0.001% by weight or less, and Si: 0.6 to 1.4% by weight. Examples of the AS-based alloy having Al of 0.1 to less than 2.0% by weight are AS21 and the like. The AS21 is a magnesium-based alloy, for example, containing Al: 1.4 to 2.6% by weight, Zn: 0.1% by weight or less, Cu: 0.15% by weight or less, Mn: 0.35 to 0.60% by weight, Ni: 0.001% by weight, and Si: 0.6 to 1.4% by weight.

Examples of the AM-based alloy are AM60, AM100 and the like. The AM60 is a magnesium-based alloy, for example, containing Al: 5.5 to 6.5% by weight, Zn: 0.22% by weight or less, Cu: 0.35% by weight or less, Mn: 0.13% by weight or more, Ni: 0.03% by weight or less, and Si: 0.5% by weight or less. The AM100 is a magnesium-based alloy, for example, containing Al: 9.3 to 10.7% by weight, Zn: 0.3% by weight or less, Cu: 0.1% by weight or less, Mn: 0.1 to 0.35% by weight, Ni: 0.01% by weight or less, and Si: 0.3% by weight or less.

Examples of the ZK-based alloy are ZK40, ZK60 and the like. The ZK40 is a magnesium-based alloy, for example, containing Zn: 3.5 to 4.5% by weight, and Zr: 0.45% by weight or more. The ZK60 is a magnesium-based alloy, for example, containing Zn: 4.8 to 6.2% by weight, and Zr: 0.45% by weight or more.

It is difficult to obtain sufficient strength with only magnesium, but if the above-described chemical compositions are containd, preferable strength can be obtained.

The present invention can be applied to produce a wrought product obtained by subjecting a drawn material to plastic processing, such as an eyeglass frame, a reinforcing frame of portable electronic equipment or others, a screw and the like.

### Brief Description of the Drawings

Figs. 1(a) and 1(b) are graphs showing whether forging processing can be carried out when forging processing is carried out while changing reduction in height at various temperatures, wherein Fig. 1(a) shows a drawn material and Fig. 1(b) shows extruded material;
Figs. 2(a) and 2(b) are graphs showing whether swaging processing can be carried out when swaging processing is carried out while changing cross section reduction ratio at various temperatures, wherein Fig. 2 (a) shows a drawn material and Fig. 2(b) shows extruded material; and
Figs. 3(a) and 3(b) are graphs showing whether bending processing can be carried out when bending processing is carried out while changing a ratio R/t of bending radius R and thickness t of material to be processed at various temperatures, wherein Fig. 3(a) shows a drawn material and Fig. 3(b) shows rolled material.

### Best Mode for Carrying Out the Invention

Embodiments of the present invention will be explained below.

### (Embodiment 1)

Extruded materials (φ4.0 mm, φ3.0 mm) of magnesium-based alloy (material corresponding to ASTM symbol AZ31) containing Al: 3.0% by weight, Zn: 1.0% by weight, Mn: 0.15% by weight, and balance comprising Mg and impurities were prepared. The extruded material of φ4.0 mm was subjected to drawing processing to φ3.0 mm at the temperature of about 160°C and processing degree of cross section reduction ratio per one pass of 20% or less (temperature rising speed to 160°C is about 10°C/sec, linear speed is 16 m/sec). After the drawing processing, thermal treatment of 350°C x 15 min was carried out. As a result, distortion caused at the time of drawing processing was eliminated and structure was equally divided finely by recrystallization.

The obtained drawn material of φ3.0 mm and the extruded material of φ3.0 mm which was not subj ected to drawing processing were cut into pieces of 3 mm length as test pieces. These test pieces were subjected to forging processing in a line axis direction with various reductions in height. At that time, the test pieces were heated to various temperatures in a range of 100°C to 250°C, and forging processing was carried out. Then, it was checked whether forging processing could be carried out. A result thereof is shown in Figs. 1(a) and 1(b). In Figs. 1(a) and 1 (b), ○ shows that forging processing could be carried out, × shows that a crack or the like was generated and forging processing could not be carried out, and Δ shows that forging processing could be carried out but heating temperature was high and there was a problem in terms of lifetime of a mold. In Figs. 1(a) and 1(b), an equation (1) is T = 3r₁+150 and an equation (2) is T = 3r₁+10. In the equations (1) and (2), T represents heating temperature, and r₁ represents reduction in height.

As shown in Fig. 1(a), when drawn material is to be subjected to forging processing, if the drawn material is heated to the temperature T°C which satisfies T ≥ 3r₁+10 with respect to reduction in height of r₁ (%), forging processing could be carried out. That is, when drawn material is used, it can be found that even if it is heated to temperature lower than 250°C, forging processing can sufficiently be carried out. Especially forging processing having reduction in height of about 20 to 30%, forging processing could be carried out sufficiently even at temperature that satisfied T < 3r₁+150. When the drawn material was heated to 250°C, forging processing could be carried out with reduction in height in a range of 20 to 80%, but if lifetime of a mold is taken into consideration, it is preferable that the drawn material is heated to lower than 250°C.

On the other hand, when extruded material which was not subjected to drawing processing was subjected to forging processing as shown in Fig. 1(b), the extruded material could not be processed without heating the extruded material to temperature that satisfied T ≥ 3r₁+150 with respect to reduction in height of r₁ (%). Especially in the case of forging processing with reduction in height of more than 40% which is industrially effective processing, it can be found that the material must be heated to 250°C or higher.

Similar tests were carried out using magnesium-based alloys having different compositions. That is, after extruded material was subjected to drawing processing, drawn material subjected to thermal treatment was subjected to forging processing in the linear axis direction at various temperatures in a range of 100 to 250°C with various reductions in height. Compositions of magnesium-based alloys subjected to the test will be shown below.

A magnesium-based alloy containing Al: 1.2% by weight, Zn: 0.4% by weight, Mn: 0.3% by weight, and balance comprising Mg and impurities (material corresponding to ASTM symbol AZ10)

A magnesium-based alloy containing Al: 6.4% by weight, Zn: 1.0% by weight, Mn: 0.28% by weight, and balance comprising Mg and impurities (material corresponding to ASTM symbol AZ61)

A magnesium-based alloy containing Al: 9.0% by weight, Zn: 0.7% by weight, Mn: 0.1% by weight, and balance comprising Mg and impurities (material corresponding to ASTM symbol AZ91)

A magnesium-based alloy containing Al: 1.9% by weight, Mn: 0.45% by weight, Si: 1.0% by weight, and balance comprising Mg and impurities (material corresponding to ASTM symbol AS21)

A magnesium-based alloy containing Al: 4.2% by weight, Mn: 0.50% by weight, Si: 1.1% by weight, and balance comprising Mg and impurities (material corresponding to ASTM symbol AS41)

A magnesium-based alloy containing Al: 6.1% by weight, Mn: 0.44% by weight, and balance comprising Mg and impurities (material corresponding to ASTM symbol AM60)

A magnesium-based alloy containing Zn: 5.5% by weight, Zr: 0.45% by weight, and balance comprising Mg and impurities (material corresponding to ASTM symbol ZK60)

With any of the above samples, if it was heated to temperature T°C that satisfied T≥3r₁+10 with respect to reduction in height of r₁ (%), forging processing could be carried out and even if it was heated to lower than 250°C, it could be processed sufficiently.

### (Embodiment 2)

The drawn material (material corresponding to ASTM symbol AZ31) of φ3.0 mm prepared under the same drawing conditions as those of the embodiment 1, and the extruded material (material corresponding to ASTM symbol AZ31) of φ3.0 mm which was not subjected to drawing processing were subjected to swaging processing. The swaging processing was carried out in such a manner that test pieces were heated to various temperatures in a range of 100°C to 250°C, and cross section reduction ratio was changed so that the following seven kinds of diameters could be obtained: i.e., φ2.7 mm (cross section reduction ratio 19%), φ2.4 mm (cross section reduction ratio 36%), φ2.3 mm (cross section reduction ratio 41.2%), φ2.1 mm (cross section reduction ratio 51%), φ1.9 mm (cross section reduction ratio 59.9%), φ1.6 mm (cross section reduction ratio 71.6%) and φ1.4 mm (cross section reduction ratio 78.2%). Then, it was checked whether swaging processing could be carried out. A result thereof is shown in Figs. 2(a) and 2(b). In Figs. 2(a) and 2(b), ○ shows that swaging processing could be carried out, × shows that a crack or the like was generated and swaging processing could not be carried out, and Δ shows that swaging processing could be carried out but heating temperature was high and there was a problem in terms of lifetime of a mold. In Figs. 2(a) and 2(b), an equation (3) is T = 3r₂+150 and an equation (4) is T = 3r₂-30. In the equations (3) and (4), T represents heating temperature, and r₂ represents cross section reduction ratio.

As shown in Fig. 2 (a), when drawn material is to be subj ected to swaging processing, if the drawn material is heated to the temperature T°C which satisfies T ≥ 3r₂-30 with respect to cross section reduction ratio r₂ (%), swaging processing could be carried out. That is, when drawn material is used, it can be found that even if it is heated to temperature lower than 250°C, swaging processing can sufficiently be carried out. Especially swaging processing having cross section reduction ratio of about 20 to 30%, swaging processing could be carried out sufficiently even at temperature T°C that satisfied T < 3r₂+150. When the drawn material was heated to 250°C, swaging processing could be carried out with cross section reduction ratio in a range of 20 to 80%, but if lifetime of a mold is taken into consideration, it is preferable that the drawn material is heated to lower than 250°C.

On the other hand, when extruded material which was not subjected to drawing processing was subjected to swaging processing as shown in Fig. 2(b), the extruded material could not be processed without heating the extruded material to temperature T°C that satisfied T ≥ 3r₂+150 even if the cross section reduction ratio r₂ is about 20 to 30%. Especially when the cross section reduction ratio is 40% or more, the swaging processing could not be carried out without heating the material to 250°C or higher.

Similar tests were carried out using magnesium-based alloys having different compositions. That is, after extruded material was subjected to the same drawing processing as that of the embodiment 1, drawn material subjected to thermal treatment was subj ected to swaging processing with various cross section reduction ratio and at various temperatures in a range of 100 to 250°C so that the above seven kinds of diameters could be obtained. As the magnesium-based alloys, the following materials having the same compositions as those shown above were used, i.e., a material corresponding to AZ10, a material corresponding to AZ61, a material corresponding to AZ91, a material corresponding to AS21, a material corresponding to AS41, a material corresponding to AM60 and a material corresponding to ZK60.

As a result of the test, with any of the samples, swaging processing could be carried out by heating the drawing material to the temperature T°C that satisfied T ≥ 3r₂-30 with respect to cross section reduction ratio r₂ (%), and the drawing material could sufficiently be processed even if the heating temperature is lower than 250°C.

### (Embodiment 3)

A drawn material of φ3.0 mm (material corresponding to ASTM symbol AZ31) prepared under the same drawing conditions as those of the embodiment 1 was further subjected to drawing processing (temperature 160°C, cross section reduction ratio per one pass was about 15 to 18%, temperature rising speed to 160°C was about 10°C/sec, linear speed was 20 m/sec), and a linear material having rectangular cross sectional shape (thickness t 1 mm x width 3 mm) was obtained. This linear material was subjected to thermal treatment of 350°C x 15 min, and test pieces were obtained. Further, a rolled material having the same component (material corresponding to ASTM symbol AZ31) as that used in the embodiment 1 and thickness t of 1 mm was prepared, it was cut into width of 3 mm as test pieces.

The test pieces of drawn material of thickness t 1 mm x width 3 mm, and rolled material of thickness t 1 mm x width 3 mm were subjected to bending processing with various bending radii R. The bending processing was carried out by heating the test pieces at various temperature in a range of 20 to 250°C. Then, it was checked whether bending processing could be carried out. Figs. 3 (a) and 3 (b) show a result thereof. In Figs. 3(a) and 3(b), ○ shows that bending processing could be carried out, × shows that a crack or the like was generated and bending processing could not be carried out, and Δ shows that bending processing could be carried out but heating temperature was high and there was a problem in terms of lifetime of a mold. In Figs. 3(a) and 3(b), an equation (5) is T = -250R/t+250 and an equation (6) isT=-250R/t+500. In the equations (5) and (6), T represents heating temperature, R represents a bending radius and t represents a thickness of test piece.

As shown in Fig. 3 (a), when drawn material is to be subj ected to bending processing, if a ratio R/t of the bending radius R (mm) and thickness t (mm) of the test piece satisfied 0.1 ≤ R/t ≤ 1.0, the bending processing could be carried out by heating the test piece to temperature T°C that satisfied T ≥ -250R/t+250. Especially when the R/t was more than 1.0 and less than 2.0, the bending processing could sufficiently be carried out even if the temperature satisfied T < -250R/t+500, specifically, the temperature was 20°C that is around the room temperature. Further, the bending processing could sufficiently be carried out at 20°C even if the R/t was 2.0. That is, when drawn material is used, it can be found that the bending processing can sufficiently be carried out even if the heating temperature is lower than 250°C. When the drawn material was heated to 250°C, bending processing could be carried out with the R/t in a range of 1.0 to 2.0, but if lifetime of a mold is taken into consideration, it is preferable that the drawn material is heated to lower than 250°C.

On the other hand, when rolled material which was not subjected to drawing processing was subjected to bending processing as shown in Fig. 3(b), the rolled material could not be processed without heating the rolled material to temperature T°C that satisfied T ≥ -250R/t+500 even if the R/t was 1.0 or more. In the case of severe processing in which the R/t was 0.5 or less, bending processing could not be carried out even if the rolled material was heated to 250°C.

Similar tests were carried out using magnesium-based alloys having different compositions. That is, after extruded material was subjected to the same drawing processing as that of the embodiment 1, drawn material was subjected to drawing processing to obtain rectangular cross section and then, was subjected to thermal treatment. This drawn material was subjected to bending processing with various bending radii so that the R/t falls in a range of 0.1 to 2.0 and at various temperatures in a range of 20 to 250°C. As the magnesium-based alloys, the following materials having the same compositions as those shown above were used, i.e., a material corresponding to AZ10, a material corresponding to AZ61, a material corresponding to AZ91, a material corresponding to AS21, a material corresponding to AS41, a material corresponding to AM60 and a material corresponding to ZK60.

As a result of the test, any of samples could be sufficiently subjected to bending processing by heating the samples to the temperature T°C satisfying T ≥ -250R/t+250 when 0.1 ≤ Rt ≤ 1.0. In addition, any of samples could be sufficiently subjected to bending processing even in the case where the temperature T°C is smaller than -250R/t+500 when 1.0 < R/t ≤ 1.9 or in the case where the temperature T°C is 20°C which is around room temperature when R/t is 1.0 or more. As described above, any of the samples could be sufficiently subjected to bending processing even if heating was carried out at less than 250°C.

### Industrial Applicability

As explained above, according to the producing method of magnesium-based alloy wrought product of the present invention, there is an excellent effect that plastic processing can be carried out at processing temperature of lower than 250°C by using a drawn material obtained by drawing processing. Therefore, according to the invention, it is unnecessary to increase a temperature as high as 250°C or more at the time of plastic processing, unlike the conventional technique in which extruded material or rolled material is subjected to plastic processing as it is. Therefore, it is possible to increase lifetime of material to be processed such as a mold and a roll, and to obtain a wrought product of magnesium-based alloy with excellent productivity.

## Claims

1. A method of producing a magnesium-based alloy wrought product, the method comprising:
providing a drawn magnesium-based alloy material having an average crystal particle diameter of 10µm or less obtained by drawing processing, and
subjecting the drawn material to plastic processing at a processing temperature (T°C) of lower than 250°C to form the wrought product,
wherein the plastic processing is one of:
(1) forging processing with a reduction in height (r₁%) of 20 ≤ r₁ < 80 at a processing temperature that also satisfies 3r₁+150 > T ≥ 3r₁+10,
(2) swaging processing with cross section reduction ratio (r₂%) of 20 ≤ r₂ < 80 at a processing temperature that also satisfies 3r₂+150 > T ≥ 3r₂-30, and
(3) bending processing with R/t of 2.0 or less, where t is the thickness of the material in mm and R is the bending radius in mm during bending, at a processing temperature that also satisfies the conditions:
250 > T ≥ 250-250R/t when 0.1 ≤ R/t ≤ 1.0,
500-250R/t ≥ T > 0 when 1.0 < R/t ≤ 1.9, and
25 ≥ T > 0 when 1.9 < R/t ≤ 2.0.

2. The method of claim 1, wherein the magnesium-based alloy contains 0.1 to 12% by weight Al.

3. The method of claim 2, wherein the magnesium-based alloy contains at least one of 0.1 to 2.0% by weight Mn, 0.1 to 5.0% by weight Zn and 0.1 to 5.0% by weight Si.

4. The method of claim 1, wherein the magnesium-based alloy contains 0.1 to 10% by weight Zn and 0.1 to 2.0% by weight Zr.

## Patentansprüche

1. Verfahren zur Herstellung eines gehämmerten Produktes einer Magnesiumbasislegierung, wobei das Verfahren enthält:
Bereistellen eines gezogenen Magnesiumbasislegierungs-Materials, das einen durchschnittlichen Kristallpartikeldurchmesser von höchstens 10 µm hat und das man durch ziehende Bearbeitung erhält, und
Unterziehen des gezogenen Materials einer plastischen Bearbeitung bei einer Bearbeitungstemperatur (T°C) von weniger als 250°C, um das gehämmerte Produkt auszubilden,
wobei die plastische Bearbeitung durch eine der folgenden Bearbeitungen erfolgt:
(1) eine Schmiedebearbeitung mit einer Verringerung der Höhe (r₁%) von 20 ≤ r₁ ≤ 80 bei einer Bearbeitungstemperatur, die zudem 3r₁+150 > T ≥ 3r₁+10 erfüllt,
(2) eine Hämmerbearbeitung mit einem Querschnittsverringerungsanteil (r₂%) von 20 ≤ r₂ < 80 bei einer Bearbeitungstemperatur, die zudem 3r₂+150 > D ≥ 3r₂-30 erfüllt, und
(3) eine Biegebearbeitung mit R/t von höchstens 2,0, wobei t die Dicke des Materials in mm und R der Biegeradius in mm während das Biegens ist, bei einer Bearbeitungstemperatur, die zudem folgende Bedingungen erfüllt:
250 > T ≥ 250-250R/t, wenn 0,1 ≤ R/t ≤ 1,0,
500-250R/t ≥ T > 0, wenn 1,0 < R/t ≤ 1,9, und
25 ≥ T > 0, wenn 1,9 < R/t ≤ 2,0.

2. Verfahren nach Anspruch 1, bei dem die Magnesiumbasislegierung 0,1 bis 12 Gew.-% Al enthält.

3. Verfahren nach Anspruch 2, bei dem die Magnesiumbasislegierung 0,1 bis 2,0 Gew.-% Mn und/oder 0,1 bis 5,0 Gew.-% Zn und/oder 0,1 bis 5,0 Gew.-% Si enthält.

4. Verfahren nach Anspruch 1, bei dem die Magnesiumbasislegierung 0,1 bis 10 Gew.-% Zn und 0,1 bis 2,0 Gew.-% Zr enthält.

## Revendications

1. Procédé de production d'un produit ouvré en alliage à base de magnésium, le procédé comprenant :
la fourniture d'un matériau en alliage à base de magnésium étiré ayant un diamètre moyen de particule cristalline de 10 µm ou moins obtenu par une mise en forme par étirage, et
l'exposition du matériau étiré à une mise en forme plastique à une température de mise en forme (T°C) inférieure à 250°C pour former le produit ouvré,
où la mise en forme plastique est l'une de :
(1) une mise en forme par forgeage avec une réduction de hauteur (r₁%) de 20 ≤ r₁ < 80 à une température de mise en forme qui satisfait aussi 3r₁+150 > T ≥ 3r₁+10,
(2) une mise en forme par estampage avec un taux de réduction de la section transversale (r₂%) de 20 ≤ r₂ < 80 à une température de mise en forme qui satisfait aussi 3r₂+150 > T ≥ 3r₂-30, et
(3) une mise en forme par pliage avec R/t de 2,0 ou moins, où t est l'épaisseur du matériau en mm et R est le rayon de pliage en mm pendant le pliage, à une température de mise en forme qui satisfait aussi les conditions :
250 > T ≥ 250-250R/t quand 0,1 ≤ R/t ≤ 1,0,
500-250R/t ≥ T > 0 quand 1,0 < R/t ≤ 1,9, et
25 ≥ T > 0 quand 1,9 < R/t ≤ 2,0.

2. Procédé selon la revendication 1 où l'alliage à base de magnésium contient 0,1 à 12 % en masse de Al.

3. Procédé selon la revendication 2 où l'alliage à base de magnésium contient au moins l'un de 0,1 à 2,0 % en masse de Mn, 0,1 à 5,0 % en masse de Zn et 0,1 à 5,0 % en masse de Si.

4. Procédé selon la revendication 1 où l'alliage à base de magnésium contient 0,1 à 10 % en masse de Zn et 0,1 à 2,0 % en masse de Zr.
